

# UNITED STATES PATENT OFFICE.

OTTO RÖHM, OF DARMSTADT, GERMANY, ASSIGNOR, BY MESNE ASSIGNMENTS, TO  
THE CHEMICAL FOUNDATION, INC., A CORPORATION OF DELAWARE.

## PROCESS FOR TANNING WITH IRON SALTS.

1,426,322.

Specification of Letters Patent. Patented Aug. 15, 1922.

No Drawing.

Application filed June 13, 1917. Serial No. 174,643.

To all whom it may concern:

Be it known that I, OTTO RÖHM, a subject of the King of Wurttemberg, residing at No. 4-6 Weiterstädterstrasse, in the city of 5 Darmstadt, Grand Duchy of Hessia, German Empire, have invented an Improvement in Processes for Tanning with Iron Salts; and I do hereby declare that the following is a full, clear, and exact description 10 of the same.

In tanning with the usual iron salts, such as ferric chloride, or sulphate of iron, it has been noticed that the leather, if, after it has 15 been tanned, it is treated with water, will allow the tanning principle to issue from the grain. This appearance is known as "bleeding." As a consequence the grain becomes defective, and the leather, being insufficiently tanned, can become hard.

With the object of preventing this bleeding, the leather, after it has been allowed 20 to remain in a moist condition for several days, or without such treatment, can be neutralized with carbonic acid, or boric acid salts, or alkalies, or alkaline earths, but this 25 is a difficult task. It is particularly necessary to take care not to carry the neutralization too far, because otherwise the grain will become brittle. Only by exercising the 30 greatest care is it possible to entirely avoid this mistake.

Now it has been found that this bleeding of the leather can be easily prevented, if, instead of one of the usual inorganic salts, 35 formate of iron alone, or together with inorganic iron salts is used for the tanning process.

The solution can be either acid or basic. Leather produced in this way can be immediately treated with water, that is, without being first stored, and without being neutralized, and does not lose its tanning.

For example 100 parts of depilated skins are treated with 150 parts of water, 3 parts 40 of common salt and 2 parts of formic acid, and then with 30 parts  $\frac{2}{3}$  basic formate of iron, with gradual strengthening.

Or 100 parts of depilated skins are treated with 150 parts of water, 30 parts of common 45 salt and 2 parts of hydrochloric acid and

then with 15 parts of  $\frac{2}{3}$  basic chloride of iron and 15 parts of  $\frac{2}{3}$  basic formate of iron, with gradual strengthening.

Further it has been found that the bleeding is also prevented if the moist leather 55 taken out of the tanning liquor is treated with the solution of a salt of lower fatty acids. Of special advantage, for example, are the calcium salts of formic or acetic acid. In this case no loss of tanning principle occurs on washing the leather, and a previous neutralization is unnecessary.

According to this process, for example, 100 parts of leather tanned with  $\frac{2}{3}$  basic solution of ferric chloride are agitated for 65 half an hour in 200 parts of water and 8 parts of formate of calcium, whereafter it is washed with water, greased, dyed and trimmed.

It has indeed been proposed to treat ferro 70 leather, after it has been tanned with solutions of neutral salts of alkalies, such as sodium sulphate and sodium chloride. The salts of fatty acids however are much superior to such an organic sodium salts. 75

What I claim and desire to secure by Letters Patent of the United States is:

1. The process of tanning consisting in subjecting the leather to the action of iron salts, then treating the same with a neutralizing agent without rendering the grain of the leather brittle, and finally subjecting the leather thus treated to the action of formate of iron. 80

2. The process of tanning leather consisting in treating depilated skins with water, sodium chloride and formic acid and finally with basic formate of iron. 85

3. The process of tanning leather consisting in first subjecting the depilated skins to 90 a moistening action by the use of water, then treating the moist skins with sodium chloride and an acid, and then further treating the skins with basic chloride of iron and basic formate of iron. 95

4. The process of tanning leather consisting in subjecting the skins to the action of a solution of an iron salt, a lower fatty acid and an organic iron salt.

OTTO RÖHM.